



US011746465B2

(12) **United States Patent**  
**Tai et al.**

(10) **Patent No.:** **US 11,746,465 B2**  
(45) **Date of Patent:** **Sep. 5, 2023**

(54) **PROCESS FOR FORMING A SYNTHETIC LEATHER**

(71) Applicants: **Dow Global Technologies LLC**,  
Midland, MI (US); **Rohm and Haas Company**, Collegeville, PA (US)

(72) Inventors: **Xiangyang Tai**, Shanghai (CN);  
**Zhaohui Qu**, Shanghai (CN); **Ruijun Zhao**, Shanghai (CN); **Yunlong Guo**, Shanghai (CN); **Xiaoyi Pang**, Shanghai (CN)

(73) Assignee: **The Dow Chemical Company**,  
Midland, MI (US)

(\*) Notice: Subject to any disclaimer, the term of this patent is extended or adjusted under 35 U.S.C. 154(b) by 0 days.

(21) Appl. No.: **17/267,958**

(22) PCT Filed: **Aug. 21, 2018**

(86) PCT No.: **PCT/CN2018/101462**

§ 371 (c)(1),  
(2) Date: **Feb. 11, 2021**

(87) PCT Pub. No.: **WO2020/037486**

PCT Pub. Date: **Feb. 27, 2020**

(65) **Prior Publication Data**

US 2021/0172115 A1 Jun. 10, 2021

(51) **Int. Cl.**  
**D06N 3/02** (2006.01)  
**D06N 3/14** (2006.01)  
(Continued)

(52) **U.S. Cl.**  
CPC ..... **D06N 3/02** (2013.01); **D06M 15/09** (2013.01); **D06M 23/00** (2013.01);  
(Continued)

(58) **Field of Classification Search**

CPC ..... D06N 3/02; D06N 3/0086; D06N 3/14;  
D06M 15/09; D06M 23/00; D06M  
15/564

See application file for complete search history.

(56) **References Cited**

U.S. PATENT DOCUMENTS

3,294,724 A 12/1966 Axelrood  
3,410,817 A 11/1968 McClellan, Jr. et al.  
(Continued)

FOREIGN PATENT DOCUMENTS

CN 102757540 A 10/2012  
CN 104179030 A 12/2014  
(Continued)

OTHER PUBLICATIONS

English translation of WO 2014/077403 (Year: 2014).\*  
X. Michael Liu et al., Journal of Chromatography A, 1104 (2006) 145-153.

Primary Examiner — Robert S Walters, Jr.

(74) Attorney, Agent, or Firm — Boyle Fredrickson, S.C.

(57) **ABSTRACT**

A process of making a synthetic leather includes (i) first, contacting a textile with an aqueous solution containing a cationic hydroxyethylcellulose polymer to form a modified textile component; (ii) subsequently, impregnating the modified textile component with an aqueous polyurethane dispersion externally stabilized with an anionic surfactant; and (iii) precipitating the polyurethane in the modified textile component. And a synthetic leather formed by the process.

**13 Claims, 3 Drawing Sheets**



|      |                    |                                                                                        |                  |         |                               |
|------|--------------------|----------------------------------------------------------------------------------------|------------------|---------|-------------------------------|
| (51) | <b>Int. Cl.</b>    |                                                                                        | 6,231,926 B1     | 5/2001  | Ronzani et al.                |
|      | <i>D06N 3/00</i>   | (2006.01)                                                                              | 7,306,825 B2     | 12/2007 | Mobley et al.                 |
|      | <i>D06M 23/00</i>  | (2006.01)                                                                              | 2009/0263431 A1  | 10/2009 | Fugmann et al.                |
|      | <i>D06M 15/09</i>  | (2006.01)                                                                              | 2013/0266624 A1  | 10/2013 | Tonani et al.                 |
|      | <i>D06M 15/564</i> | (2006.01)                                                                              | 2013/0288551 A1  | 10/2013 | Irnich et al.                 |
| (52) | <b>U.S. Cl.</b>    |                                                                                        | 2014/0302734 A1  | 10/2014 | Irnich et al.                 |
|      | CPC .....          | <i>D06N 3/0086</i> (2013.01); <i>D06N 3/14</i> (2013.01); <i>D06M 15/564</i> (2013.01) | 2015/0275421 A1  | 10/2015 | Cardinali et al.              |
|      |                    |                                                                                        | 2015/0284902 A1  | 10/2015 | Bhattacharjee et al.          |
|      |                    |                                                                                        | 2015/0299945 A1* | 10/2015 | Gu ..... D06N 3/144 428/319.3 |

|                       |                         |                              |
|-----------------------|-------------------------|------------------------------|
| (56)                  | <b>References Cited</b> | FOREIGN PATENT DOCUMENTS     |
| U.S. PATENT DOCUMENTS |                         |                              |
|                       |                         |                              |
| 3,412,054 A           | 11/1968                 | Milligan et al.              |
| 3,527,653 A *         | 9/1970                  | Erwin ..... C08J 9/28 521/64 |
| 4,737,156 A *         | 4/1988                  | Tambor ..... D06P 5/08 8/606 |
| 5,539,021 A           | 7/1996                  | Pate et al.                  |
| 5,688,842 A           | 11/1997                 | Pate, III et al.             |
| 5,959,027 A           | 9/1999                  | Jakubowski et al.            |
| EP                    |                         |                              |
|                       |                         |                              |
| JP                    | 0399198 A2              | 11/1990                      |
| RU                    | S52-151703 A            | 12/1977                      |
| TW                    | 2001181 C1              | 10/1993                      |
| WO                    | 201414901 A             | 4/2014                       |
| WO                    | 2011/137565 A1          | 11/2011                      |
| WO                    | 2014059593 A1           | 4/2014                       |
| WO                    | WO-2014077403 A1 *      | 5/2014 ..... C11D 1/835      |
| WO                    | 2018/037039 A1          | 3/2018                       |

\* cited by examiner



Figure 1



Figure 2



Figure 3



Figure 4



Figure 5



Figure 6



Figure 7



Figure 8



Figure 9

## PROCESS FOR FORMING A SYNTHETIC LEATHER

## BACKGROUND

The present disclosure relates to a process for forming a synthetic leather.

A growing number of applications exist for synthetic leather, including clothing, footwear, bags and luggage, home upholstery, and automobile seats. Synthetic leather can exhibit similar performance and handfeeling to natural leather, but synthetic leather provides the added advantages of being animal-friendly and less expensive to produce. Synthetic leather is conventionally produced by impregnating a polyurethane solution containing an organic solvent (e.g., dimethyl formamide (DMF)) into a textile and then adding water to precipitate the polyurethane and form a porous polyurethane matrix. The porous structure gives the synthetic leather the soft handfeeling that is similar to natural leather. DMF is hazardous to manufacturers, processors, consumers, and the environment.

Attempts have been made to form synthetic leather without organic solvent by utilizing aqueous polyurethane. Known is the foaming (or frothing) of the aqueous polyurethane dispersion, and applying the foamed polyurethane dispersion onto a textile, and then drying the textile. However, the relatively high viscosity required by the aqueous polyurethane dispersion in order to provide stability to the foam bubbles (during application and drying) impedes impregnation of the aqueous polyurethane dispersion into the textile. Broken air bubbles lower the porosity of the resulting polyurethane matrix, which deteriorates the soft handfeeling of the resulting synthetic leather.

The art recognizes the need for the production of synthetic leather which avoids the use of organic solvents. The art further recognizes the need for aqueous-based production synthetic leather.

## SUMMARY

The present disclosure provides a process. The process includes (i) first, contacting a textile with an aqueous solution containing a cationic hydroxyethylcellulose polymer to form a modified textile component; (ii) subsequently, impregnating the modified textile component with an aqueous polyurethane dispersion externally stabilized with an anionic surfactant; and (iii) precipitating the polyurethane in the modified textile component.

The present disclosure also provides a synthetic leather formed by the process.

## BRIEF DESCRIPTION OF THE DRAWINGS

FIG. 1 is a number of scanning electron microscope (SEM) micrographs of Comparative Sample 1.

FIG. 2 is a number of SEM micrographs of Comparative Sample 2.

FIG. 3 is a number of SEM micrographs of Example 3, in accordance with an embodiment of the present disclosure.

FIG. 4 is a number of SEM micrographs of Example 4, in accordance with an embodiment of the present disclosure.

FIG. 5 is a number of SEM micrographs of Example 5, in accordance with an embodiment of the present disclosure.

FIG. 6 is a number of SEM micrographs of Example 6, in accordance with an embodiment of the present disclosure.

FIG. 7 is a number of SEM micrographs of Example 7, in accordance with an embodiment of the present disclosure.

FIG. 8 is a number of SEM micrographs of Example 8, in accordance with an embodiment of the present disclosure.

FIG. 9 is a number of SEM micrographs of Example 9, in accordance with an embodiment of the present disclosure.

## DEFINITIONS

Any reference to the Periodic Table of Elements is that as published by CRC Press, Inc., 1990-1991. Reference to a group of elements in this table is by the new notation for numbering groups.

For purposes of United States patent practice, the contents of any referenced patent, patent application or publication are incorporated by reference in their entirety (or its equivalent US version is so incorporated by reference) especially with respect to the disclosure of definitions (to the extent not inconsistent with any definitions specifically provided in this disclosure) and general knowledge in the art.

The numerical ranges disclosed herein include all values from, and including, the lower and upper value. For ranges containing explicit values (e.g., 1 or 2, or 3 to 5, or 6, or 7), any subrange between any two explicit values is included (e.g., 1 to 2; 2 to 6; 5 to 7; 3 to 7; 5 to 6; etc.).

Unless stated to the contrary, implicit from the context, or customary in the art, all parts and percents are based on weight and all test methods are current as of the filing date of this disclosure.

The term "alkyl" refers to an organic radical derived from an aliphatic hydrocarbon by deleting one hydrogen atom therefrom. An alkyl group may be a linear, branched, cyclic or a combination thereof. Nonlimiting examples of suitable alkyls include methyl, ethyl, n-propyl, i-propyl, n-butyl, t-butyl, i-butyl (or 2-methylpropyl), etc. In an embodiment, the alkyl has from 1 to 8, or 12, or 20, or 22 carbon atoms.

An "alkylene" (also known as an "alkene"), is an unsaturated, aliphatic hydrocarbon with one or more carbon-carbon double bonds.

An "anion" is a negatively charged ion.

An "arylene" is an aromatic hydrocarbon that has had a hydrogen atom removed from two ring carbon atoms. Non-limiting examples of arylanes include o-phenylene and benzene-1,2-diyl.

The terms "blend" or "polymer blend," as used herein, is a blend of two or more polymers. Such a blend may or may not be miscible (not phase separated at molecular level). Such a blend may or may not be phase separated. Such a blend may or may not contain one or more domain configurations, as determined from transmission electron spectroscopy, light scattering, x-ray scattering, and other methods known in the art.

An "cation" is a positively charged ion.

The term "composition" refers to a mixture of materials which comprise the composition, as well as reaction products and decomposition products formed from the materials of the composition.

The terms "comprising," "including," "having" and their derivatives, are not intended to exclude the presence of any additional component, step or procedure, whether or not the same is specifically disclosed. In order to avoid any doubt, all compositions claimed through use of the term "comprising" may include any additional additive, adjuvant, or compound, whether polymeric or otherwise, unless stated to the contrary. In contrast, the term "consisting essentially of" excludes from the scope of any succeeding recitation any other component, step, or procedure, excepting those that are not essential to operability. The term "consisting of" excludes any component, step, or procedure not specifically

delineated or listed. The term "or," unless stated otherwise, refers to the listed members individually as well as in any combination. Use of the singular includes use of the plural and vice versa.

An "externally stabilized polyurethane dispersion" is an emulsion containing polyurethane that substantially fails to have an ionic or nonionic hydrophilic pendant groups on or within the polyurethane, and thus requires the addition of a surfactant (such as an anionic surfactant) to stabilize the polyurethane dispersion. Nonlimiting examples of externally stabilized polyurethane dispersions are described in U.S. Pat. Nos. 5,539,021; 5,688,842 and 5,959,027, each herein incorporated in its entirety by reference.

"Fabric" is a woven or non-woven (such as knitted) structure formed from individual fibers or yarn.

"Fiber" and like terms refer to an elongated column of entangled filaments. Fiber diameter can be measured and reported in a variety of fashions. Generally, fiber diameter is measured in denier per filament. Denier is a textile term which is defined as the grams of the fiber per 9000 meters of that fiber's length. Monofilament generally refers to an extruded strand having a denier per filament greater than 15, usually greater than 30. Fine denier fiber generally refers to fiber having a denier of 15 or less. Microdenier (aka micro-fiber) generally refers to fiber having a diameter not greater than 100 micrometers.

"Filament" and like terms refer to a single, continuous strand of elongated material having generally round cross-section and a length to diameter ratio of greater than 10.

A "hydrocarbon" is a compound that contains only hydrogen and carbon atoms. The hydrocarbon can be (i) branched or unbranched, (ii) saturated or unsaturated (iii) cyclic or acyclic, and (iv) any combination of (i)-(iii). Nonlimiting examples of hydrocarbons include alkanes, alkenes, and alkynes.

An "internally stabilized polyurethane dispersion" is an emulsion containing polyurethane that is stabilized through the incorporation of hydrophilic pendant groups (such as anionically hydrophilic pendant groups) on the polyurethane, which is dispersed in the liquid medium. Typically, dihydroxyalkylcarboxylic acids such as described by U.S. Pat. No. 3,412,054, incorporated in its entirety herein by reference, are used to make anionic internally stabilized polyurethane dispersions. A nonlimiting example of a suitable monomer used to make an anionic internally stabilized polyurethane dispersion is dimethylolpropionic acid (DMPA).

An "interpolymer" is a polymer prepared by the polymerization of at least two different monomers. This generic term includes copolymers, usually employed to refer to polymers prepared from two different monomers, and polymers prepared from more than two different monomers, e.g., terpolymers, tetrapolymers, etc.

A "knitted fabric" is formed from intertwining yarn or fibers in a series of connected loops either by hand, with knitting needles, or on a machine. The fabric may be formed by warp or weft knitting, flat knitting, and circular knitting. Nonlimiting examples of suitable warp knits include tricot, raschel powernet, and lacing. Nonlimiting examples of suitable weft knits include circular, flat, and seamless (which is often considered a subset of circular knits).

"Nonwoven" refers to a web or a fabric having a structure of individual fibers or threads which are randomly interlaid, but not in an identifiable manner as is the case of a knitted fabric.

An "olefin-based polymer" or "polyolefin" is a polymer that contains more than 50 weight percent polymerized

olefin monomer (based on total amount of polymerizable monomers), and optionally, may contain at least one comonomer. A nonlimiting examples of an olefin-based polymer is ethylene-based polymer.

5 A "polymer" is a compound prepared by polymerizing monomers, whether of the same or a different type, that in polymerized form provide the multiple and/or repeating "units" or "mer units" that make up a polymer. The generic term polymer thus embraces the term homopolymer, usually 10 employed to refer to polymers prepared from only one type of monomer, and the term copolymer, usually employed to refer to polymers prepared from at least two types of monomers. It also embraces all forms of copolymer, e.g., random, block, etc. The terms "ethylene/α-olefin polymer" 15 and "propylene/α-olefin polymer" are indicative of copolymer as described above prepared from polymerizing ethylene or propylene respectively and one or more additional, polymerizable α-olefin monomer. It is noted that although a polymer is often referred to as being "made of" one or more specified monomers, "based on" a specified monomer or monomer type, "containing" a specified monomer content, or the like, in this context the term "monomer" is understood 20 to be referring to the polymerized remnant of the specified monomer and not to the unpolymerized species. In general, polymers herein are referred to as being based on "units" that are the polymerized form of a corresponding monomer.

25 "Woven" refers to a web or a fabric having a structure of individual fibers or threads which are interlaid in a pattern in an identifiable manner. A nonlimiting example of a woven fabric is a knitted fabric.

30 "Yarn" is a continuous length of twisted or otherwise entangled filaments that can be used in the manufacture of woven or knitted fabrics.

### 35 Test Methods

Average pore size is determined by measuring the area of about 100 pores randomly, using image analysis software on a scanning electron microscope (SEM) micrograph, such as 40 Leica QWin software available from Leica Microsystems AG of Wetzlar, Germany, and calculating the mean average pore size.

Density is measured in accordance with ASTM D792, Method B. The result is recorded in grams per cubic 45 centimeter (g/cc).

Mean volume average particle size is measured using a Beckman Coulter LS 230 Laser Light Scattering Particle Sizer, available from Beckman Coulter Corporation.

50 Viscosity is measured using a Brookfield Viscometer Model, and a Brookfield RV-DV-II-Pro viscometer spindle #62 under 30 rmp, at 25° C. for the polyurethane dispersion and at 25° C. for the cationic hydroxyethylcellulose solution. Gel Permeation Chromatography (GPC)

55 A high temperature gel permeation chromatography (GPC) system, equipped with Robotic Assistant Deliver (RAD) system is used for sample preparation and sample injection. The concentration detector is an Infra-red detector (IR-5) from Polymer Char Inc. (Valencia, Spain). Data collection is performed using a Polymer Char DM 100 Data 60 acquisition box. The carrier solvent is 1,2,4-trichlorobenzene (TCB). The system is equipped with an on-line solvent degas device from Agilent. The column compartment is operated at 150° C. The columns are four Mixed A LS 30 cm, 20 micron columns. The solvent is nitrogen-purged 65 1,2,4-trichlorobenzene (TCB) containing approximately 200 ppm 2,6-di-t-butyl-4-methylphenol (BHT). The flow rate is 1.0 mL/min, and the injection volume is 200 µL. A "2

## 5

mg/mL" sample concentration is prepared by dissolving the sample in N<sub>2</sub> purged and preheated TCB (containing 200 ppm BHT), for 2.5 hours at 160° C., with gentle agitation.

The GPC column set is calibrated by running twenty narrow molecular weight distribution polystyrene standards. The molecular weight (MW) of the standards ranges from 580 g/mol to 8,400,000 g/mol, and the standards are contained in six "cocktail" mixtures. Each standard mixture has at least a decade of separation between individual molecular weights. The equivalent polypropylene molecular weights of each PS standard are calculated by using following equation, with reported Mark-Houwink coefficients for polypropylene (Th. G. Scholte, N. L. J. Meijerink, H. M. Schoffeleers, & A. M. G. Brands, *J. Appl. Polym. Sci.*, 29, 3763-3782 (1984)) and polystyrene (E. P. Otocka, R. J. Roe, N. Y. Hellman, & P. M. Muglia, *Macromolecules*, 4, 507 (1971)):

$$M_{PP} = \left( \frac{K_{PS} M_{PS}^{a_{PS}+1}}{K_{PP}} \right)^{\frac{1}{a_{PP}+1}}, \quad (\text{Eq } 1)$$

where M<sub>PP</sub> is PP equivalent MW, M<sub>PS</sub> is PS equivalent MW, log K and a values of Mark-Houwink coefficients for PP and PS are listed below.

| Polymer       | a     | log K  |
|---------------|-------|--------|
| Polypropylene | 0.725 | -3.721 |
| Polystyrene   | 0.702 | -3.900 |

A logarithmic molecular weight calibration is generated using a fourth order polynomial fit as a function of elution volume. Number average and weight average molecular weights are calculated according to the following equations:

$$M_n = \frac{\sum_i Wf_i}{\sum_i (Wf_i / M_i)}, \quad (\text{Eq } 2)$$

$$M_w = \frac{\sum_i (Wf_i * M_i)}{\sum_i (Wf_i)}, \quad (\text{Eq } 3)$$

where Wf<sub>i</sub> and M<sub>i</sub> are the weight fraction and molecular weight of elution component i, respectively.

## DETAILED DESCRIPTION

The present disclosure provides a process. The process includes (i) first, contacting a textile with an aqueous solution containing a cationic hydroxyethylcellulose polymer to form a modified textile component; (ii) subsequently, impregnating the modified textile component with an aqueous polyurethane dispersion; and (iii) precipitating the polyurethane in the modified textile component.

The present disclosure provides another process. The process includes (i) first, contacting a textile with an aqueous solution containing a cationic hydroxyethylcellulose polymer to form a modified textile component; (ii) subsequently, impregnating the modified textile component with an aqueous polyurethane dispersion externally stabilized with an anionic surfactant; and (iii) precipitating the polyurethane in the modified textile component.

## 6

In an embodiment, the process includes (iv) forming a synthetic leather.

## (1) Contacting a Textile with an Aqueous Solution

The process includes the step of contacting a textile with an aqueous solution containing a cationic hydroxyethylcellulose polymer to form a modified textile component.

## A. Textile

A textile is contacted with an aqueous solution containing a cationic hydroxyethylcellulose polymer. A "textile" is a flexible material composed of a network of natural fibers, artificial fibers, and combinations thereof. Textile includes fabric and cloth. The textile may be woven or nonwoven. In an embodiment, the textile is a nonwoven textile. Nonlimiting examples of artificial fibers include polyesters, polyamides, acrylics, polyolefins, polyvinyl chlorides, polyvinylidene chlorides, polyvinyl alcohols, and combinations thereof. Nonlimiting examples of suitable natural fibers include cotton, wool, hemp, and combinations thereof. In an embodiment, the textile is a nonwoven textile containing polyamide/polyethylene fibers.

In an embodiment, the textile is a microfiber nonwoven textile. A "microfiber" textile is a fabric containing fiber having a diameter not greater than 100 micrometers.

In an embodiment, the textile has a density from 0.20 g/cc, or 0.25 g/cc to 0.27 g/cc, or 0.30 g/cc, or 0.31 g/cc, or 0.32 g/cc, or 0.35 g/cc, or 0.40 g/cc, or 0.50 g/cc.

In an embodiment, the textile contains fibers having a size from 0.1 denier, or 0.3 denier, or 1 denier, or 2 denier, or 3 denier to 4 denier, or 5 denier, or 6 denier, or 7 denier, or 8 denier, or 9 denier, or 10 denier. In another embodiment, the textile contains fibers having a size equal to or less than 10 denier.

In an embodiment, the textile has a thickness from 0.5 mm, or 1.0 mm to 1.5 mm, or 2.0 mm.

In an embodiment, the textile is a nonwoven textile having one, some, or all of the following properties:

(a) a density from 0.20 g/cc, or 0.25 g/cc to 0.32 g/cc, or 0.35 g/cc; and/or

(b) a fiber size from 1 denier, or 3 denier to 5 denier; and/or

(c) a thickness from 0.5 mm, or 1.0 mm to 1.5 mm, or 2.0 mm.

The textile may comprise two or more embodiments disclosed herein.

## B. Aqueous Solution

The process includes contacting the textile with an aqueous solution containing a cationic hydroxyethylcellulose polymer. A "cationic hydroxyethylcellulose polymer" (or "CH Polymer") is a hydroxyethylcellulose polymer having a cationic group bound to its polymeric backbone. Nonlimiting examples of suitable cationic groups include a quaternary ammonium cation group and a quaternary phosphonium cation group. The CH Polymer is water soluble.

In an embodiment, the aqueous solution contains a CH Polymer with a quaternary ammonium cation group. In a further embodiment, the aqueous solution contains a CH Polymer with a quaternary ammonium cation group with the following Structure (A):



wherein n refers to the number of repeating units of the cationic hydroxyethylcellulose;  
 x refers to the number of repeating units of ethylene oxide ( $\text{CH}_2\text{CH}_2\text{O}$ ); and  
 y refers to the number of repeating units of quaternary ammonium cation group.

In an embodiment, n of Structure (A) is a positive integer from 200 to 10,000.

In an embodiment, x of Structure (A) is an integer from 0 to 30.

In an embodiment, y of Structure (A) is a positive integer from 1 to 10.

In an embodiment, in Structure (A):

n is a positive integer from 200 to 10,000;

x is an integer from 0 to 30; and

y is a positive integer from 1 to 10.

Nonlimiting examples of suitable CH Polymers with a quaternary ammonium cation group with Structure (A) include those sold under the trade name UCARE™ JR, available from The Dow Chemical Company, including UCARE™ JR 125, UCARE™ JR 400, and UCARE™ JR 30M.

In an embodiment, the CH Polymer has a weight average molecular weight (Mw) from 100,000 Daltons, or 250,000 Daltons, or 500,000 Daltons, or 1,000,000 Daltons to 2,000,000 Daltons, or 3,000,000 Daltons. Not wishing to be bound by any particular theory, it is believed that a CH Polymer with a Mw higher than 3,000,000 Daltons would be too slow to disperse in the aqueous medium to exhibit greater coalescence. In other words, a CH Polymer with a Mw higher than 3,000,000 Daltons will be too slow to dispersion in the aqueous medium, which results in ineffective precipitation of the polyurethane. In another embodiment, the CH Polymer has a Mw from 100,000 Daltons, or 250,000 Daltons, or 290,000 Daltons to 900,000 Daltons, or 1,000,000 Daltons.

In an embodiment, the CH Polymer contains from 0.5 wt %, or 1.0 wt %, or 1.5 wt % to 2.2 wt %, or 2.5 wt %, or 3.0 wt %, or 5.0 wt % nitrogen, based on the total weight of the CH Polymer. In a further embodiment, the CH Polymer contains from 1.5 wt % to 2.2 wt % nitrogen, based on the total weight of the CH Polymer.

In an embodiment, an aqueous solution containing 2 wt % CH Polymer has a viscosity from 50 cP, or 75 cP, or 100 cP, or 200 cP, or 300 cP to 500 cP, or 1,000 cP, or 5,000 cP, or 10,000 cP, or 20,000 cP, or 30,000 cP, or 35,000 cP.

In an embodiment, the aqueous solution contains from 0.20 wt %, or 0.25 wt %, or 0.40 wt %, or 0.50 wt %, or 0.60 wt % to 0.80 wt %, or 0.90 wt %, or 1.00 wt %, or 1.20 wt %, or 1.50 wt %, or 2.0 wt %, or 3.0 wt % of the CH Polymer.

In an embodiment, the aqueous solution contains, consists essentially of, or consists of, from 0.20 wt %, or 0.25 wt %, or 0.40 wt %, or 0.50 wt %, or 0.60 wt % to 0.80 wt %, or 0.90 wt %, or 1.00 wt %, or 1.20 wt %, or 1.50 wt %, or 2.0 wt %, or 3.0 wt % of the CH Polymer; and a reciprocal amount of water, or from 97 wt %, or 98 wt %, or 98.50 wt %, or 98.80 wt %, or 99.00 wt %, or 99.10 wt %, or 99.20 wt % to 99.40 wt %, or 99.50 wt %, or 99.60 wt %, or 99.70 wt %, or 99.75 wt %, or 99.80 wt % water, based on the total weight of the aqueous solution.

The aqueous solution may optionally contain an additive. A nonlimiting example of a suitable additive is a softening agent, such as silicone oil.

In an embodiment, the aqueous solution consists essentially of the CH Polymer and water. In another embodiment, the aqueous solution consists of the CH Polymer and water.

In an embodiment, the process includes selecting an aqueous solution having one or both of the following properties:

- 20 (a) the CH Polymer has a Mw from 100,000 Dalton, or 250,000 Dalton, or 500,000 Dalton, or 1,000,000 Dalton to 2,000,000 Dalton, or 3,000,000 Dalton; and/or
- (b) the CH Polymer contains from 0.5 wt %, or 1.0 wt %, or 1.5 wt % to 2.2 wt %, or 2.5 wt %, or 3.0 wt %, or 5.0 wt % nitrogen; and/or
- (c) a viscosity from 50 cP, or 75 cP, or 100 cP, or 200 cP, or 300 cP to 500 cP, or 1,000 cP, or 5,000 cP, or 10,000 cP, or 20,000 cP, or 30,000 cP, or 35,000 cP, when measured in an aqueous solution containing 2 wt % of the CH Polymer.

It is understood that the sum of the components in each of the aqueous solutions disclosed herein, including the foregoing aqueous solution, yields 100 wt %.

In an embodiment, the aqueous solution excludes free inorganic salts. A “free” salt is a salt compound that is not bound to a polymeric backbone. Free inorganic salts, such as NaCl and Ca(NO<sub>3</sub>)<sub>2</sub>, are problematic because they form pollutants in waste water. By excluding free inorganic salts, the present process advantageously avoids the need for waste water treatment to remove pollutants.

35 The aqueous solution is void of, or substantially void of organic solvents. An “organic solvent” is an organic compound that can dissolve a solute and displays a heightened flammability and vapor pressure (i.e., greater than 0.1 mm of Hg), such as dimethyl formamide (DMF).

The textile is contacted with the aqueous solution to form a modified textile component. A “modified textile component” is a textile with fibers that are in contact with the CH Polymer.

50 Nonlimiting examples of suitable procedures for contacting the textile with aqueous solution of CH Polymer include dipping, immersing, brushing, spraying or doctor blading. In an embodiment, the textile is immersed in the aqueous solution. In a further embodiment, the textile is immersed in the aqueous solution for a duration from 30 seconds, or 1 minute to 90 seconds, or 2 minutes, or 5 minutes, or 10 minutes, the aqueous solution having a temperature from 20° C., or 23° C. to 25° C., or 30° C.

55 After the contacting, the modified textile component may have excess aqueous solution or water. In an embodiment, excess aqueous solution or water are removed from modified textile component by passing the modified textile component through rollers, such as rubber rollers. In an embodiment, after the contacting, the modified textile component is passed through a two-roller machine, through an impregnation padder, or is hand-rolled. Not wishing to be bound by any particular theory, it is believed that the rollers/padder

also facilitate homogenous penetration of the aqueous solution into the textile, such that all, or substantially all, of the fibers of the textile are contacted with the aqueous solution.

In an embodiment, after the contacting, the modified textile component is dried in an oven. In an embodiment, the modified textile component is dried in an oven at a temperature from 70° C., or 80° C., or 90° C. to 100° C., or 110° C., or 120° C., or 150° C. for a duration from 1 minute, or 5 minutes, or 10 minutes, or 15 minutes to 20 minutes, or 30 minutes, or 40 minutes, or 60 minutes. In an embodiment, the drying removes all, or substantially all, of the water from the modified textile component.

In an embodiment, before the drying, the modified textile component contains from 25 wt %, or 28 wt %, or 30 wt %, or 35 wt %, or 40 wt %, or 44 wt %, or 45 wt %, or 50 wt % to 72 wt %, or 75 wt %, or 80 wt % of the aqueous solution, based on the total weight of the modified textile component.

The contacting step may comprise two or more embodiments disclosed herein.

(2) Impregnating the Modified Textile Component with an Aqueous Polyurethane Dispersion and Precipitating the Polyurethane in the Modified Textile Component

The process includes impregnating the modified textile component with an aqueous polyurethane dispersion. In an embodiment, the process includes impregnating the modified textile component with an aqueous polyurethane dispersion externally stabilized with an anionic surfactant.

The process includes precipitating the polyurethane in the modified textile component.

A. Aqueous Polyurethane Dispersion

The modified textile component is impregnated with an aqueous polyurethane dispersion.

An “aqueous polyurethane dispersion” (or “PUD”) is an emulsion containing polyurethane particles, an anionic moiety, and water. The PUD may be an internally stabilized PUD or an externally stabilized PUD.

In an embodiment, the PUD is an internally stabilized PUD. In an internally stabilized PUD, the anionic moiety is incorporated within the polyurethane polymeric backbone. Nonlimiting examples of suitable monomers having anionic moieties include aliphatic, cycloaliphatic, araliphatic, or aromatic carboxylic acids and sulfonic acids that include at least one alcoholic hydroxyl group or at least one primary or secondary amino group. A nonlimiting example of a suitable monomer having an anionic moiety is dimethylolpropionic acid (DMPA). A nonlimiting example of a PUD that is internally stabilized with DMPA is Primal™ U-51, available from The Dow Chemical Company.

In an embodiment, the PUD is an externally stabilized PUD. In an externally stabilized PUD, the anionic moiety is incorporated into the dispersion as an anionic surfactant. Nonlimiting examples of suitable anionic surfactants include sulfonates, sulfates, and carboxylates. In an embodiment, the PUD is externally stabilized with a sulfonate surfactant. A nonlimiting example of a PUD that is externally stabilized with a sulfonate surfactant is SYNTEGA™ YS3000, available from The Dow Chemical Company.

The aqueous polyurethane dispersion is void of, or substantially void of organic solvents. In an embodiment, the PUD contains from 0 wt %, or greater than 0 wt %, or 0.1 wt %, or 0.3 wt % to 0.5 wt %, or 1 wt % organic solvent, based on the total weight of the PUD. It is understood that the PUD may or may not include residual organic solvent

from the PU synthesis. In an embodiment, the PUD has no detectable organic solvent present (i.e., “void” of an organic solvent).

In an embodiment, the PUD is prepared by reacting a polyurethane/urea/thiourea prepolymer with a chain-extending reagent in an aqueous medium and in the presence of a stabilizing amount of an external anionic surfactant. The polyurethane/urea/thiourea prepolymer is prepared by contacting a high molecular weight organic compound having at least two active hydrogen atoms with a polyisocyanate, and under such conditions to ensure that the prepolymer is terminated with at least two isocyanate groups.

In an embodiment, the polyisocyanate is an organic diisocyanate, and may be aromatic, aliphatic, or cycloaliphatic, or a combination thereof. Nonlimiting examples of suitable diisocyanates include those disclosed in U.S. Pat. No. 3,294,724, column 1, lines 55 to 72, and column 2, lines 1 to 9, incorporated herein by reference, as well as U.S. Pat. No. 3,410,817, column 2, lines 62 to 72, and column 3, lines 1 to 24, also incorporated herein by reference. Nonlimiting examples of suitable organic diisocyanate include 4,4'-diisocyanatodiphenylmethane, 2,4'-diisocyanatodiphenylmethane, isophorone diisocyanate, p-phenylene diisocyanate, 2,6 toluene diisocyanate, polyphenyl polymethylene polyisocyanate, 1,3-bis(isocyanatomethyl)cyclohexane, 1,4-diisocyanatocyclohexane, hexamethylene diisocyanate, 1,5-naphthalene diisocyanate, 3,3'-dimethyl-4,4'-biphenyl diisocyanate, 4,4'-diisocyanatodicyclohexylmethane, 2,4'-diisocyanatodicyclohexylmethane, and 2,4-toluene diisocyanate, or combinations thereof.

An “active hydrogen group” is a group that reacts with an isocyanate group to form a urea group, a thiourea group, or a urethane group as illustrated by the general reaction:



where X is O, S, NH, or N; and R and R' are connecting groups that may be aliphatic, aromatic, cycloaliphatic, or combinations thereof.

The “high molecular weight organic compound” with at least two active hydrogen atoms is an organic compound with a weight average molecular weight (Mw) of at least 500 Daltons. The high molecular weight organic compound having at least two active hydrogen atoms may be a polyol (e.g., diol), a polyamine (e.g., diamine), a polythiol (e.g., dithiol), or a mixture thereof (e.g., an alcohol-amine, a thiol-amine, or an alcohol-thiol). The polyol, polyamine, or polythiol compound may be primarily a diol, triol, or polyol having greater active hydrogen functionality, or a mixture thereof. It is understood that these mixtures may have an overall active hydrogen functionality that is slightly below 2, for example, due to a small amount of monol in a polyol mixture.

In an embodiment, the high molecular weight organic compound having at least two active hydrogen atoms is a polyalkylene glycol ether, or thioether, or polyester polyol, or polythiol having the general Structure (B):



## 11

where each R is independently an alkylene radical; R' is an alkylene or an arylene radical; each X is independently S or O; and n and n' each is a positive integer.

In an embodiment, the NCO:XH ratio, where X is O or S, is from 1.1:1, or 1.2:1 to 5:1.

In an embodiment, the high molecular weight organic compound having at least two active hydrogen atoms has a weight average molecular weight (Mw) of at least 500 Daltons, or from 500 Daltons, or 750 Daltons, or 1,000 Daltons to 3,000 Daltons, or 5,000 Daltons, or 10,000 Daltons, or 20,000 Daltons.

In an embodiment, the high molecular weight organic compound having at least two active hydrogen atoms is a polyalkylene ether glycol or a polyester polyol. Nonlimiting examples of suitable polyalkylene ether glycols are polyethylene ether glycols, poly-1,2-propylene ether glycols, polytetramethylene ether glycols, poly-1,2-dimethylethylene ether glycols, poly-1,2-butylene ether glycol, and poly-decamethylene ether glycols. Nonlimiting examples of suitable polyester polyols include polybutylene adipate, caprolactone based polyester polyol, and polyethylene terephthalate (PET).

The polyurethane prepolymer may be prepared by a batch process or a continuous process. In an embodiment, a stoichiometric excess of a diisocyanate and a polyol can be introduced in separate streams into a static or an active mixer at a temperature suitable for controlled reaction of the reagents, typically from 40° C. to 100° C. A catalyst may be used to facilitate the reaction of the reagents, such as an organotin catalyst (e.g., stannous octoate). The reaction is generally carried to substantial completion in a mixing tank to form the prepolymer. In an embodiment, the PUD is prepared as disclosed in U.S. Pat. No. 5,539,021, column 1, lines 9 to 45, the entire content of which is herein incorporated by reference.

When making the PUD, the prepolymer may be extended by water solely, or may be extended using a chain extender, such as those known in the art. The chain extender may be any isocyanate reactive diamine or amine having another isocyanate reactive group and a molecular weight of from 60 g/mol to 450 g/mol. In an embodiment, the chain extender is selected from an aminated polyether diol; piperazine, aminoethylethanolamine, ethanamine, ethylenediamine and mixtures thereof. In an embodiment, the amine chain extender is dissolved in the water used to make the dispersion.

The external stabilizing surfactant is an anionic surfactant. Nonlimiting examples of suitable anionic surfactants include sulfonates, phosphates, carboxylates, and combinations thereof. In an embodiment, the anionic surfactant is a sulfonate, such as sodium dodecyl benzene sulfonate, sodium dodecyl sulfonate, sodium dodecyl diphenyl oxide disulfonate, sodium n-decyl diphenyl oxide disulfonate, isopropylamine dodecylbenzenesulfonate, and sodium hexyl diphenyl oxide disulfonate. In a further embodiment, the anionic surfactant is sodium dodecyl benzene sulfonate.

In an embodiment, a flowing stream containing the prepolymer is merged with a flowing stream containing water with sufficient shear to form the PUD. An amount of a stabilizing surfactant is also present, either in the stream containing the prepolymer, in the stream containing the water, or in a separate stream. The relative rates of the stream containing the prepolymer (R2) and the stream containing the water (R1) are preferably such that the polydispersity of the emulsion (the ratio of the volume average diameter and the number average diameter of the particles or droplets, or D<sub>v</sub>/D<sub>n</sub>) is less than 5, or less than 3,

## 12

or less than 2, or less than 1.5, or less than 1.3; or the mean volume average particle size is less than 2 microns, or less than 1 micron, or less than 0.5 micron, or less than 0.3 micron. The PUD may be prepared in a continuous process without phase inversion or stepwise distribution of an internal phase into an external phase.

In an embodiment, the anionic surfactant is used as a concentrate in water. In this case, a stream containing the anionic surfactant is first merged with a stream containing the prepolymer to form a prepolymer/surfactant mixture. The PUD can be prepared in this single step. In another embodiment, a stream containing the prepolymer and the anionic surfactant can be merged with a water stream to dilute the anionic surfactant and to create the PUD.

The PUD may optionally contain an additive. Nonlimiting examples of suitable additives include rheological modifiers such as a thickeners; fillers, UV stabilizers, deformers, crosslinking agents, acrylic latex, and polyolefin latex. When the PUD contains another polymer such as an acrylic latex or a polyolefin latex, a dried film formed from the PUD contains at least 30 volume percent polyurethane, based on the total volume of the dried film.

In an embodiment, the PUD has a solids content from 5 wt %, or 10 wt %, or 11 wt %, or 15 wt %, or 20 wt %, or 21 wt to 30 wt %, or 40 wt %, or 50 wt %, or 55 wt %, or 60 wt %, or 65 wt %, based on the total weight of the PUD. In another embodiment, the PUD has a solids content from 30 wt %, or 35 wt %, or 40 wt %, or 45 wt %, or 50 wt % to 55 wt %, or 60 wt %, based on the total weight of the PUD.

In an embodiment, the PUD has a Viscosity at 25° C. from 100 cP, or 150 cP, or 200 cP, or 300 cP, or 400 cP, or 500 cP, or 550 cP to 570 cP, or 600 cP, or 700 cP, or 800 cP, or 900 cP, or 1,000 cP, or 5,000 cP, or 10,000 cP.

In an embodiment, the PUD has a density from 0.99 g/cc, or 1.00 g/cc, or 1.05 g/cc to 1.10 g/cc, or 1.20 g/cc, or 1.30 g/cc.

In an embodiment, the PUD has a mean volume average particle size from 100 nm, or 250 nm, or 300 nm, or 350 nm, or 370 nm to 380 nm, or 400 nm, or 450 nm, or 800 nm.

In an embodiment, the process includes selecting a sulfonate surfactant as the anionic surfactant. In a further embodiment, process includes selecting a PUD that is a polyether based aqueous polyurethane dispersion that is externally stabilized with a sulfonate surfactant. The PUD has one, some, or all of the following properties:

- (a) a solids content from 10 wt %, or 11 wt %, or 15 wt %, or 20 wt %, or 21 wt %, or 30 wt %, or 35 wt % to 40 wt %, or 50 wt %, or 55 wt %, or 60 wt %; and/or
- (b) a Viscosity at 25° C. from 100 cP, or 150 cP, or 200 cP, or 300 cP, or 400 cP, or 500 cP, or 550 cP to 570 cP, or 600 cP, or 700 cP, or 800 cP, or 900 cP, or 1,000 cP; and/or
- (c) a density from 0.99 g/cc, or 1.00 g/cc, or 1.05 g/cc to 1.10 g/cc, or 1.20 g/cc; and/or
- (d) a mean volume average particle size from 300 nm, or 350 nm, or 370 nm to 380 nm, or 400 nm; and/or
- (e) an organic solvent content of 0 wt %.

It is understood that the sum of the components in each of the PUDs disclosed herein, including the foregoing PUD, yields 100 wt %.

In an embodiment, the PUD excludes free inorganic salts.

The PUD may be mixed with other dispersions so long as the dispersion mixture is easily and quickly coagulated as described below. Other polymer dispersions or emulsions that may be useful when mixed with the PUD include polymers such as polyacrylates, polyisoprene, polyolefins,

## 13

polyvinyl alcohol, nitrile rubber, natural rubber and co-polymers of styrene and butadiene. In an embodiment, the PUD is used alone (i.e., not mixed with any other polymeric dispersion or emulsion).

The PUD may comprise two or more embodiments disclosed herein.

## B. Impregnating and Precipitating

The present process includes impregnating the modified textile component with the PUD. The impregnation step occurs after the contacting step with the aqueous solution containing CH Polymer. Nonlimiting examples of suitable impregnation processes include dipping, immersing, brushing, spraying or doctor blading. In an embodiment, the modified textile component is immersed in the PUD. In a further embodiment, the modified textile component is immersed in the PUD for a duration from 30 seconds, or 1 minute to 90 seconds, or 2 minutes, or 5 minutes, or 10 minutes, the aqueous solution having a temperature from 20° C., or 23° C. to 25° C., or 30° C.

Not wishing to be bound by any particular theory, it is believed that by first contacting the textile with the aqueous solution containing a CH Polymer, the impregnation of the PUD is more homogenous throughout the textile because the anion group within the PUD is attracted to the cation group within the CH Polymer (which is present throughout the textile following the contacting step).

The present process includes precipitating the polyurethane in the modified textile component. During and/or after impregnation, the cationic group within the CH Polymer, and further within the modified textile component, reacts with the anionic group within the PUD to deactivate the surfactant and cause coagulation. In other words, the cationic group within the cationic hydroxyethylcellulose polymer and the anionic group within the PUD for an ionic pair to form a precipitate. For example, the quaternary ammonium cation group of the CH Polymer reacts with the anionic group of the PUD to stabilize (i.e., neutralize) the anionic charge of the surfactant in the PUD, resulting in the PUD losing its stability and precipitating the polyurethane.

The polyurethane is precipitated in and on the textile. Polyurethane that is "precipitated in" the textile is located between opposing surfaces of the textile. Polyurethane that is "precipitated on" the textile is located on a surface of the textile.

In an embodiment, the process includes precipitating the polyurethane in the textile during impregnation. In a further embodiment, the process includes precipitating the polyurethane in the textile during and after impregnation.

In an embodiment, during impregnation and any subsequent drying, the molar ratio of the cationic group within the CH Polymer and the anionic group within the PUD (i.e., the "Cation:Anion Ratio") is from 0.1, or 0.2, or 0.3, or 0.4, or 0.5 to 1.8, or 2, or 3, or 5, or 10. The Cation:Anion ratio is the ratio of the number of moles of cation groups (e.g., quaternary ammonium cation groups) to the number of moles of anion groups (e.g., from the anionic surfactant). Not wishing to be bound by any particular theory, it is believed that a Cation:Anion Ratio of less than 0.1 would cause insufficient coalescence. In other words, too few cation moieties will result in incomplete neutralization of the anion moieties. Incomplete neutralization of the anion moieties on the surfactant prevents the PUD from losing its stability, thereby preventing precipitation of the polyurethane. Additionally, it is believed that a Cation:Anion Ratio of greater than 10 would result in free CH Polymer (which is water soluble). The free CH Polymer would run off the textile with waste water, which must then be disposed.

## 14

The impregnating step may comprise two or more embodiments disclosed herein.

The precipitating step may comprise two or more embodiments disclosed herein.

## 5 (3) Forming a Synthetic Leather

In an embodiment, the process includes forming a synthetic leather.

A "synthetic leather" is a textile having fibers suspended within a porous polyurethane matrix. In other words, a 10 synthetic leather has a porous polyurethane matrix that at least partially encapsulates, or fully encapsulates, the fibers of a textile. The polyurethane is located in the textile and on the textile surface. A synthetic leather is not naturally occurring in nature.

15 In an embodiment, after the impregnating, the synthetic leather is passed through a two-roller machine, through an impregnation padder, or is hand-rolled. Not wishing to be bound by any particular theory, it is believed that the rollers/padder facilitate homogenous penetration of the PUD into the modified textile component, such that the entire modified textile component is impregnated with the PUD. In other words, the PUD is impregnated throughout the entire thickness of the synthetic leather.

20 In an embodiment, after the impregnating, the synthetic leather is exposed to water. In a further embodiment, after impregnating, the textile is immersed in water at a temperature from 90° C., or 100° C. to 110° C. for a duration from 1 minute, or 2 minutes to 3 minutes, or 4 minutes, or 5 minutes, or 10 minutes, or 20 minutes. In another embodiment, after impregnating, the synthetic leather is exposed to 25 steam at a temperature of 100° C. for a duration of from 1 minute, or 2 minutes to 3 minutes, or 4 minutes, or 5 minutes, or 10 minutes, or 20 minutes, or 30 minutes. Not wishing to be bound by any particular theory, it is believed that exposure to steam causes faster precipitation (i.e., coagulation) of the polyurethane into the modified textile component. Additionally, it is believed that exposure to steam aids in the impregnation of the PUD into the modified 30 textile component.

35 In an embodiment, after the impregnating, the textile is exposed to a heated aqueous solution containing a cationic hydroxyethylcellulose polymer. The aqueous solution, and further the cationic hydroxyethylcellulose polymer may be any aqueous solution and CH Polymer disclosed herein. In a further embodiment, after impregnating, the textile is immersed in aqueous solution at from 90° C., or 100° C. to 110° C. for from 1 minute, or 2 minutes to 3 minutes, or 4 minutes, or 5 minutes, or 10 minutes, or 20 minutes. Not wishing to be bound by any particular theory, it is believed that exposure to a heated aqueous solution containing a 40 cationic hydroxyethylcellulose polymer after the impregnating enables further precipitating of the polyurethane when complete precipitation is not accomplished during the impregnating.

45 The synthetic leather has two opposing surfaces. In an embodiment, after the impregnating, each surface of the synthetic leather is covered with a polyethylene membrane (such as a plastic bag). A surface that is "covered" with a polyethylene membrane is in direct contact with the polyethylene membrane, with no intervening layers or structures between the synthetic leather surface and the polyethylene membrane. The polyethylene membrane slows the evaporation of water from the synthetic leather. After covering each surface with a polyethylene membrane, the synthetic 50 leather is dried in an oven. In an embodiment, after covering each surface with a polyethylene membrane, the synthetic leather is dried in an oven at a temperature from 80° C., or 55 60

## 15

90° C. to 100° C., or 110° C., or 120° C., or 130° C. for a duration of from 10 minutes, or 15 minutes to 20 minutes. Then, the polyethylene membranes are each removed and the synthetic leather is further dried in an oven. In embodiment, after removing the polyethylene membranes, the synthetic leather is dried in an oven at a temperature from 80° C., or 90° C. to 100° C., or 110° C., or 120° C., or 130° C. for a duration of from 10 minutes, or 15 minutes to 20 minutes, or 30 minutes, or 40 minutes, or 60 minutes. In an embodiment, the drying removes all, or substantially all of the water from the synthetic leather. 10

In an embodiment, the synthetic leather is dried in an oven. In an embodiment, the synthetic leather is dried in an oven at a temperature from 80° C., or 90° C. to 100° C., or 110° C., or 120° C., or 130° C. for a duration of from 10 minutes, or 15 minutes to 20 minutes, or 30 minutes, or 40 minutes, or 60 minutes, or 70 minutes, or 90 minutes. In an embodiment, the drying removes all, or substantially all of the water from the synthetic leather. 15

In an embodiment, the synthetic leather is washed with toluene. Washing with toluene includes immersing the synthetic leather in toluene at a temperature from 80° C., or 85° C. to 90° C., or 100° C. for a duration of from 30 minutes, or 60 minutes, or 90 minutes to 120 minutes, or 150 minutes, or 180 minutes, or 210 minutes. Not wishing to be bound by any particular theory, it is believed that the toluene wash dissolves polyethylene from textiles formed from co-spun polyamide/polyethylene fiber, resulting in a synthetic leather with polyamide fiber having a having a diameter not greater than 100 micrometers (i.e., a polyamide microfiber). 20

In an embodiment, the synthetic leather undergoes water washing, a softening treatment, and/or a coloring treatment.

In an embodiment, the synthetic leather contains from 5 wt %, or 6 wt %, or 15 wt %, or 16 wt %, or 20 wt %, or 30 wt %, or 40 wt %, or 50 wt % to 60 wt %, or 70 wt % 35 polyurethane, based on the total weight of the synthetic leather. In another embodiment, the synthetic leather contains from 20 wt %, or 30 wt %, or 40 wt %, or 50 wt to 60 wt %, or 70 wt % polyurethane, based on the total weight of the synthetic leather. 40

The synthetic leather has pores in the polyurethane matrix. A “pore” is a void volume within the polyurethane matrix. In an embodiment, the synthetic leather has an average pore size from 10 μm to 200 μm.

In an embodiment, the process includes forming a synthetic leather with a polyurethane matrix having pores, the synthetic leather having one or both of the following properties:

- (a) contains from 20 wt %, or 30 wt %, or 40 wt %, or 50 wt % to 60 wt %, or 70 wt % polyurethane, based on 50 the total weight of the synthetic leather; and/or
- (b) an average pore size from 10 μm to 200 μm.

The forming a synthetic leather step may comprise two or more embodiments disclosed herein.

The process includes (i) first, contacting a textile with an aqueous solution containing, or consisting essentially of, or consisting of, a CH Polymer to form a modified textile component; (ii) subsequently, impregnating the modified textile component with an aqueous polyurethane dispersion externally stabilized with an anionic surfactant; (iii) precipitating the polyurethane in the modified textile component; and (iv) forming a synthetic leather. In other words, steps (i) and (ii) are performed sequentially, with step (i) performed to completion before step (ii) begins. 55

In an embodiment, the process includes:

- (i) first, contacting a textile with an aqueous solution comprising a CH Polymer that is a hydroxyethylcellu-

## 16

lose polymer with a quaternary ammonium cation group to form a modified textile component, wherein the textile is a nonwoven textile having one, some, or all of the following properties:

- (a) a density from 0.20 g/cc to 0.30 g/cc, or 0.35 g/cc; and/or
- (b) a fiber size from 1 denier, or 3 denier to 5 denier; and/or
- (c) a thickness from 0.5 mm, or 1.0 mm to 1.5 mm, or 2.0 mm;

the aqueous solution has one, some, or all of the following properties:

- (a) the aqueous solution contains from 0.20 wt %, or 0.25 wt %, or 0.40 wt %, or 0.50 wt %, or 0.60 wt % to 0.80 wt %, or 0.90 wt %, or 1.00 wt %, or 1.20 wt %, or 1.50 wt %, or 2.0 wt %, or 3.0 wt % of the hydroxyethylcellulose polymer with a quaternary ammonium cation group, based on the total weight of the aqueous solution; and/or
- (b) the hydroxyethylcellulose polymer with a quaternary ammonium cation group has a Mw from 500,000 Daltons, or 1,000,000 Daltons to 2,000,000 Daltons, or 3,000,000 Daltons; and/or
- (c) the hydroxyethylcellulose polymer with a quaternary ammonium cation group contains from 0.5 wt %, or 1.0 wt %, or 1.5 wt % to 2.2 wt %, or 2.5 wt %, or 3.0 wt %, or 5.0 wt % nitrogen, based on the total weight of the hydroxyethylcellulose polymer with a quaternary ammonium cation group; and/or
- (d) the aqueous solution has a viscosity from 50 cP, or 75 cP, or 100 cP, or 200 cP, or 300 cP to 500 cP, or 1,000 cP, or 5,000 cP, or 10,000 cP, or 20,000 cP, or 30,000 cP, or 35,000 cP, when measured in an aqueous solution containing 2 wt % of the hydroxyethylcellulose polymer with a quaternary ammonium cation group;

(ii) subsequently, impregnating the modified textile component with an aqueous polyurethane dispersion externally stabilized with an anionic surfactant, wherein the PUD externally stabilized with an anionic surfactant is a polyether based aqueous polyurethane dispersion externally stabilized with a sulfonate surfactant and the PUD has one, some, or all of the following properties:

- (a) a solids content from 10 wt %, or 11 wt %, or 15 wt %, or 20 wt %, or 21 wt %, or 30 wt %, or 35 wt % to 40 wt %, or 50 wt %, or 55 wt %, or 60 wt %, based on the total weight of the PUD; and/or
- (b) a Viscosity at 25° C. from 100 cP, or 150 cP, or 200 cP, or 300 cP, or 400 cP, or 500 cP, or 550 cP to 570 cP, or 600 cP, or 700 cP, or 800 cP, or 900 cP, or 1,000 cP; and/or
- (c) a density from 0.99 g/cc, or 1.00 g/cc, or 1.05 g/cc to 1.10 g/cc, or 1.20 g/cc; and/or
- (d) a mean volume average particle size from 300 nm, or 350 nm, or 370 nm to 380 nm, or 400 nm; and/or
- (e) an organic solvent content of 0 wt %;
- (iii) precipitating the polyurethane in the modified textile component; and

## 17

(iv) forming a synthetic leather, wherein the synthetic leather has a polyurethane matrix containing pores and the synthetic leather has one, some, or all of the following properties:

(a) the synthetic leather contains from 20 wt %, or 30 wt %, or 40 wt %, or 50 wt % to 60 wt %, or 70 wt % polyurethane, based on the total weight of the synthetic leather; and/or

(b) the synthetic leather has an average pore size from 10  $\mu\text{m}$  to 200  $\mu\text{m}$ ; and/or

(c) the synthetic leather contains a polyurethane matrix distributed throughout the thickness of the textile; and/or

(d) the synthetic leather exhibits a uniform distribution of pores throughout the polyurethane matrix, and further throughout the synthetic leather; and steps (i) and (ii) are performed sequentially; and the process optionally includes one or more of the following steps:

passing the modified textile component through rollers; and/or

removing water from the modified textile component before impregnating the modified textile component with the PUD; and/or

removing water from the modified textile component by drying in an oven at a temperature from 70° C. to 120° C. for a duration of from 5 minutes to 60 minutes, before impregnating the modified textile component with the PUD; and/or

passing the synthetic leather through rollers; and/or

exposing the synthetic leather to steam at 100° C. for from 1 minute, or 2 minutes to 3 minutes, or 4 minutes, or 5 minutes, or 10 minutes, or 20 minutes, or 30 minutes; and/or

covering each surface of the synthetic leather with a polyethylene membrane, drying synthetic leather in an oven at from 80° C., or 90° C. to 100° C., or 110° C., or 120° C., or 130° C. for from 10 minutes, or 15 minutes to 20 minutes, or 30 minutes, or 40 minutes, or 60 minutes; and/or

## 18

removing the polyethylene membranes and further drying the synthetic leather in an oven at from 80° C., or 90° C. to 100° C., or 110° C., or 120° C., or 130° C. for from 10 minutes, or 15 minutes to 20 minutes, or 30 minutes, or 40 minutes, or 60 minutes; and/or

removing water from the synthetic leather, such as by drying the synthetic leather in an oven at from 80° C., or 90° C. to 100° C., or 110° C., or 120° C., or 130° C. for from 10 minutes, or 15 minutes to 20 minutes, or 30 minutes, or 40 minutes, or 60 minutes, or 70 minutes, or 90 minutes; and/or

washing the synthetic leather with toluene, such as by immersing the synthetic leather in toluene at from 80° C., or 85° C. to 90° C., or 100° C. for from 30 minutes, or 60 minutes, or 90 minutes to 120 minutes, or 150 minutes, or 180 minutes, or 210 minutes; and/or

maintaining a Cation:Anion Ratio from 0.1, or 0.3, or 0.4, or 0.5 to 1.8, or 2, or 3, or 5, or 10.

The present process may comprise two or more embodiments disclosed herein.

The present disclosure also provides a synthetic leather produced by the present process.

The present synthetic leather is useful for applications such as clothing, accessories, purses, luggage, shoes, hats, automobile interiors, and furniture.

The synthetic leather may comprise two or more embodiments disclosed herein.

By way of example, and not limitation, some embodiments of the present disclosure will now be described in detail in the following Examples.

## EXAMPLES

Materials used in the examples are provided in Table 1 below.

TABLE 1

| Material/Description | Properties                                                                                                                                                                                                                                                                     | Source                   |
|----------------------|--------------------------------------------------------------------------------------------------------------------------------------------------------------------------------------------------------------------------------------------------------------------------------|--------------------------|
| UCARE™ JR 125        | hydroxyethylcellulose polymer with a quaternary ammonium cation group polyquaternium-10; viscosity (2 wt % aqueous solution) = 75-175 cP; wt % Nitrogen = 1.5-2.2 wt % <sup>#</sup>                                                                                            | The Dow Chemical Company |
| UCARE™ JR 400        | hydroxyethylcellulose polymer with a quaternary ammonium cation group polyquaternium-10; viscosity (2 wt % aqueous solution) = 300-500 cP; wt % Nitrogen = 1.5-2.2 wt % <sup>#</sup>                                                                                           | The Dow Chemical Company |
| SYNTEGRA™ YS3000     | polyether based aqueous polyurethane dispersion externally stabilized with sulfonate surfactant solids content = 54-55 wt %*; organic solvent content* = 0 wt % density = 1.05 g/cc; pH = 7.0-8.0; Viscosity (25° C.) = 150-500 cP; mean volume average particle size = 370 nm | The Dow Chemical Company |
| Textile              | nonwoven textile containing co-spun polyamide/polyethylene fibers density = 0.27 g/cm <sup>3</sup> ; fiber size = 4 denier; thickness = 1.2-1.8 mm                                                                                                                             |                          |

\*Based on total weight of the dispersion

<sup>#</sup>Based on total weight of the hydroxyethylcellulose polymer with a quaternary ammonium cation group

19

## Comparative Sample 1 (CS 1)

A textile sample with a weight of 16.30 g is immersed for 1 minute in a PUD (SYNTEGRA™ YS3000) with a solids content of 54.5%, at room temperature (25° C.). After the textile is removed from the PUD, the textile is pressed with a Mathis impregnation gadder. After impregnating, the textile is weighed. The textile contains 16.75 g PUD. The textile is then exposed to 100° C. steam for 15 minutes, and then dried in an oven for 15 minutes at 90° C. followed by 15 minutes at 120° C. After drying, the textile is weighed. The textile contains 9.13 g polyurethane. The textile is hand-cut with a razor blade and the cross-sectional morphology of the impregnated textile is analyzed using an SEM micrograph.

FIG. 1 is a number of SEM micrographs of CS 1. As shown, the polyurethane matrix of CS 1 lacks pores.

## Comparative Sample 2 (CS 2)

A textile sample with a weight of 14.93 g is immersed for 1 minute in a PUD (SYNTEGRA™ YS3000) with a solids content of 54.5%, at room temperature (25° C.). the textile is removed from the PUD, the textile is pressed with a Werner Mathis AG, VFM 28888 two-roller machine. After rolling, the textile is weighed. The textile contains 13.97 g PUD. The textile is then dried in an oven for 15 minutes at 90° C. followed by 15 minutes at 120° C. After drying, the textile is weighed. The textile contains 7.61 g polyurethane. The textile is hand-cut with a razor blade and the cross-sectional morphology of the impregnated textile is analyzed using an SEM micrograph.

FIG. 2 is a number of SEM micrographs of CS 2. As shown, the polyurethane matrix of CS 2 lacks pores.

## Example 3 (Ex. 3)

A textile sample with a weight of 13.99 g is immersed for 1 minute in an aqueous solution containing 0.8 wt % UCARE™ JR 125 (based on the total weight of the aqueous solution) to contact the textile with the UCARE™ JR 125 solution to form a modified textile component. The aqueous solution is at room temperature (25° C.). After the modified textile component is removed from the UCARE™ JR 125 solution, the modified textile component is pressed with a Werner Mathis AG, VFM 28888 two-roller machine. The modified textile component is weighed. The modified textile component contains 11.33 g UCARE™ JR 125 solution. The modified textile component is then dried in an oven for 15 minutes at 90° C.

The dried modified textile component is immersed for 1 minute in a PUD (SYNTEGRA™ YS3000) with a solids content of 54.5%, to impregnate the modified textile component with the PUD to form a synthetic leather. The PUD is at room temperature (25° C.). After the synthetic leather is removed from the PUD, the synthetic leather is pressed with a Werner Mathis AG, VFM 28888 two-roller machine. The synthetic leather is weighed. The synthetic leather contains 18.60 g PUD. The two surfaces of the synthetic leather are covered with a polyethylene membrane (a plastic bag). The synthetic leather covered with polyethylene membranes is then dried in an oven for 15 minutes at 90° C. The polyethylene membranes are removed and the synthetic leather is dried in an oven for another 15 minutes at 90° C., and then for 15 minutes at 120° C. The synthetic leather is weighed. The synthetic leather contains 9.91 g polyurethane. The synthetic leather is hand-cut with a razor blade and the

20

cross-sectional morphology of the synthetic leather is analyzed using an SEM micrograph.

FIG. 3 is a number of SEM micrographs of Ex. 3. As shown, the polyurethane matrix of Ex. 3 contains pores. Ex. 3 exhibits good coagulation.

## Example 4 (Ex. 4)

A textile sample with a weight of 14.33 g is immersed for 1 minute in an aqueous solution containing 0.8 wt % UCARE™ JR 400 (based on the total weight of the aqueous solution) to contact the textile with the UCARE™ JR 400 solution to form a modified textile component. The aqueous solution is at room temperature (25° C.). After the modified textile component is removed from the UCARE™ JR 400 solution, the modified textile component is pressed with a Werner Mathis AG, VFM 28888 two-roller machine. The modified textile component is weighed. The modified textile component contains 12.52 g UCARE™ JR 400 solution.

20 The modified textile component is then dried in an oven for 15 minutes at 90° C.

The dried modified textile component is immersed for 1 minute in a PUD (SYNTEGRA™ YS3000) with a solids content of 54.5%, to impregnate the modified textile component with the PUD to form a synthetic leather. The PUD is at room temperature (25° C.). After the synthetic leather is removed from the PUD, the synthetic leather is pressed with a Werner Mathis AG, VFM 28888 two-roller machine. The synthetic leather is weighed. The synthetic leather contains 20.16 g PUD. The two surfaces of the synthetic leather are covered with a polyethylene membrane (a plastic bag). The synthetic leather covered with polyethylene membranes is then dried in an oven for 15 minutes at 90° C. The polyethylene membranes are removed and the synthetic leather is dried in an oven for another 15 minutes at 90° C., and then for 15 minutes at 120° C. The synthetic leather is weighed. The synthetic leather contains 11.29 g polyurethane. The synthetic leather is hand-cut with a razor blade and the cross-sectional morphology of the synthetic leather is analyzed using an SEM micrograph.

40 FIG. 4 is a number of SEM micrographs of Ex. 4. As shown, the polyurethane matrix of Ex. 4 contains pores. Ex. 4 exhibits good coagulation.

## Example 5 (Ex. 5)

A textile sample with a weight of 10.59 g is immersed for 1 minute in an aqueous solution containing 1.2 wt % UCARE™ JR 400 (based on the total weight of the aqueous solution) to contact the textile with the UCARE™ JR 400 solution to form a modified textile component. The aqueous solution is at room temperature (25° C.). After the modified textile component is removed from the UCARE™ JR 400 solution, the modified textile component is pressed with a Werner Mathis AG, VFM 28888 two-roller machine. The modified textile component is weighed. The modified textile component contains 11.25 g UCARE™ JR 400 solution. The modified textile component is then dried in an oven for 15 minutes at 90° C.

60 The dried modified textile component is immersed for 1 minute in a PUD (SYNTEGRA™ YS3000) with a solids content of 54.5%, to impregnate the modified textile component with the PUD and form a synthetic leather. The PUD is at room temperature (25° C.). After the synthetic leather is removed from the PUD, the synthetic leather is pressed with a Werner Mathis AG, VFM 28888 two-roller machine. The synthetic leather is weighed. The synthetic leather

contains 13.30 g PUD. The two surfaces of the synthetic leather are covered with a polyethylene membrane (a plastic bag). The synthetic leather covered with polyethylene membranes is then dried in an oven for 15 minutes at 90° C. The polyethylene membranes are removed and the synthetic leather is dried in an oven for another 15 minutes at 90° C., and then for 15 minutes at 120° C. The synthetic leather is weighed. The synthetic leather contains 7.16 g polyurethane. The synthetic leather is hand-cut with a razor blade and the cross-sectional morphology of the synthetic leather is analyzed using an SEM micrograph.

FIG. 5 is a number of SEM micrographs of Ex. 5. As shown, the polyurethane matrix of Ex. 5 contains pores. Ex. 5 exhibits good coagulation.

#### Example 6 (Ex. 6)

A textile sample with a weight of 0.87 g is immersed for 1 minute in an aqueous solution containing 0.4 wt % UCARE™ JR 400 (based on the total weight of the aqueous solution) to contact the textile with the UCARE™ JR 400 solution to form a modified textile component. The aqueous solution is at room temperature (25° C.). After the modified textile component is removed from the UCARE™ JR 400 solution, the modified textile component is weighed. The modified textile component contains 2.10 g UCARE™ JR 400 solution. The modified textile component is then dried in an oven for 20 minutes at 80° C.

The dried modified textile component is immersed for 1 minute in a PUD (SYNTEGRA™ YS3000) with a solids content of 54.5%, to impregnate the modified textile component with the PUD and form a synthetic leather. The PUD is at room temperature (25° C.). After the synthetic leather is removed from the PUD, the synthetic leather is pressed with a stainless steel hand roller. The synthetic leather is weighed. The synthetic leather contains 1.58 g PUD. The synthetic leather is then dried in an oven for 15 minutes at 90° C., and then for 15 minutes at 120° C. The synthetic leather is weighed. The synthetic leather contains 0.93 g polyurethane.

The synthetic leather is then washed in toluene for 3 hours at 85° C. After washing, the synthetic leather is hand-cut with a razor blade and the cross-sectional morphology of the synthetic leather is analyzed using an SEM micrograph.

FIG. 6 is a number of SEM micrographs of Ex. 6. As shown, the polyurethane matrix of Ex. 6 contains pores. Ex. 6 exhibits good coagulation.

#### Example 7 (Ex. 7)

A textile sample with a weight of 0.82 g is immersed for 1 minute in an aqueous solution containing 0.4 wt % UCARE™ JR 400 (based on the total weight of the aqueous solution) to contact the textile with the UCARE™ JR 400 solution to form a modified textile component. The aqueous solution is at room temperature (25° C.). After the modified textile component is removed from the UCARE™ JR 400 solution, the modified textile component is weighed. The modified textile component contains 1.98 g UCARE™ JR 400 solution. The modified textile component is then dried in an oven for 20 minutes at 80° C.

The dried modified textile component is immersed for 1 minute in a PUD (SYNTEGRA™ YS3000) with a solids content of 54.5%, to impregnate the modified textile component with the PUD and form a synthetic leather. The PUD is at room temperature (25° C.). After the synthetic leather is removed from the PUD, the synthetic leather is pressed

with a stainless steel hand roller. The synthetic leather is weighed. The synthetic leather contains 1.57 g PUD. The synthetic leather is then immersed in water at 100° C. for 5 minutes, and dried in an oven for 15 minutes at 90° C., and then for 15 minutes at 120° C. The c synthetic leather is weighed. The synthetic leather contains 0.83 g polyurethane.

The synthetic leather is then washed in toluene for 3 hours at 85° C. After washing, synthetic leather is hand-cut with a razor blade and the cross-sectional morphology of the synthetic leather is analyzed using an SEM micrograph.

FIG. 7 is a number of SEM micrographs of Ex. 7. As shown, the polyurethane matrix of Ex. 7 contains pores. Ex. 7 exhibits good coagulation.

15

#### Example 8 (Ex. 8)

A textile sample with a weight of 0.89 g is immersed for 1 minute in an aqueous solution containing 0.4 wt % UCARE™ JR 400 (based on the total weight of the aqueous solution) to contact the textile with the UCARE™ JR 400 solution to form a modified textile component. The aqueous solution is at room temperature (25° C.). After the modified textile component is removed from the UCARE™ JR 400 solution, the modified textile component is weighed. The modified textile component contains 2.22 g UCARE™ JR 400 solution. The modified textile component is not dried before being impregnated with a PUD.

The modified textile component is immersed for 1 minute in a PUD (SYNTEGRA™ YS3000) with a solids content of 54.5%, to impregnate the modified textile component with the PUD and form a synthetic leather. The PUD is at room temperature (25° C.). After the synthetic leather is removed from the PUD, the synthetic leather is pressed with a stainless steel hand roller. The synthetic leather is weighed. The synthetic leather contains 1.51 g PUD. The synthetic leather is then immersed in water at 100° C. for 5 minutes, and dried in an oven for 15 minutes at 90° C., and then for 15 minutes at 120° C. The synthetic leather is weighed. The synthetic leather contains 0.49 g polyurethane.

The synthetic leather is then washed in toluene for 3 hours at 85° C. After washing, synthetic leather is hand-cut with a razor blade and the cross-sectional morphology of the synthetic leather is analyzed using an SEM micrograph.

FIG. 8 is a number of SEM micrographs of Ex. 8. As shown, the polyurethane matrix of Ex. 8 contains pores. Ex. 8 exhibits good coagulation.

50

#### Example 9 (Ex. 9)

A textile sample with a weight of 11.14 g is immersed for 1 minute in an aqueous solution containing 2.0 wt % UCARE™ JR 125 (based on the total weight of the aqueous solution) to contact the textile with the UCARE™ JR 125 solution to form a modified textile component. The aqueous solution is at room temperature (25° C.). After the modified textile component is removed from the UCARE™ JR 125 solution, the modified textile component is pressed with a Werner Mathis AG, VFM 28888 two-roller machine. The modified textile component is weighed. The modified textile component contains 13.55 g UCARE™ JR 125 solution. The modified textile component is then dried in an oven for 15 minutes at 90° C.

The dried modified textile component is immersed for 1 minute in a PUD (SYNTEGRA™ YS3000), which is diluted with water to have a solids content of 21%, to form a synthetic leather. The PUD is at room temperature (25°C).

65

The synthetic leather is weighed. The synthetic leather contains 26.21 g PUD. The two surfaces of the synthetic leather are covered with a polyethylene membrane (a plastic bag). The synthetic leather covered with polyethylene membranes is then dried in an oven for 15 minutes at 90°C. The polyethylene membranes are removed and the synthetic leather is dried in an oven for another 15 minutes at 90°C, and then for 15 minutes at 120°C. The synthetic leather is weighed. The synthetic leather contains 5.83 g polyurethane. The synthetic leather is hand-cut with a razor blade and the cross-sectional morphology of the synthetic leather is analyzed using an SEM micrograph.

FIG. 9 is a number of SEM micrographs of Ex. 9. As shown, the polyurethane matrix of Ex. 9 contains pores. Ex. 9 exhibits good coagulation.

The composition of the aqueous solution and the PUD are provided in Table 2.

#### Results

The properties of each synthetic leather are provided in Table 2.

matrix, and further throughout the synthetic leather, which endows the synthetic leather with nice (i.e., soft) handfeeling, lowers the weight of the synthetic leather, and lowers the total material cost of the synthetic leather. Consequently, Examples 3-9 are suitable for synthetic leather applications such as clothing and automobile interiors.

Despite the PUD of Ex. 9 having a solids content of 21%, which is less than half the solids content of the PUD used in CS 2 (PUD solids content of 54.5 wt %), Ex. 9 surprisingly achieves a higher weight percent of polyurethane (34.4 wt %) than CS 2 (33.8 wt %) in the final synthetic leather. A higher polyurethane weight percent is advantageous in synthetic leather applications.

It is specifically intended that the present disclosure not be limited to the embodiments and illustrations contained herein, but include modified forms of those embodiments including portions of the embodiments and combinations of elements of different embodiments as come within the scope of the following claims.

TABLE 2

| Sample | Aqueous Solution <sup>1</sup> | PUD Solids Content (wt %) <sup>2</sup> | Initial Textile Weight (g) | Aqueous Solution Pick-Up (g) | Modified Textile Component wt % <sup>3</sup> | Aqueous Solution <sup>3</sup> | PUD Pick-Up (g) | Polyurethane Pick-Up (g) <sup>4</sup> | Cation:Anion Ratio | Synthetic Leather Weight After Drying (g) | Synthetic Leather Polyurethane wt % After Drying <sup>5</sup> | Porous Polyurethane Matrix |
|--------|-------------------------------|----------------------------------------|----------------------------|------------------------------|----------------------------------------------|-------------------------------|-----------------|---------------------------------------|--------------------|-------------------------------------------|---------------------------------------------------------------|----------------------------|
|        |                               |                                        |                            |                              |                                              |                               |                 |                                       |                    |                                           |                                                               |                            |
| CS 1   | —                             | 54.5                                   | 16.30                      | —                            | —                                            | —                             | 16.75           | 9.13                                  | —                  | 25.43                                     | 35.9 wt %                                                     | No                         |
| CS 2   | —                             | 54.5                                   | 14.93                      | —                            | —                                            | —                             | 13.97           | 7.61                                  | —                  | 22.54                                     | 33.8 wt %                                                     | No                         |
| Ex 3   | 0.8% UCARE™ JR 125            | 54.5                                   | 13.99                      | 11.33                        | 44.7 wt %                                    | 44.7 wt %                     | 18.60           | 9.91                                  | 0.65               | 23.9                                      | 41.5 wt %                                                     | Yes                        |
| Ex 4   | 0.8% UCARE™ JR 400            | 54.5                                   | 14.33                      | 12.52                        | 46.6 wt %                                    | 46.6 wt %                     | 20.16           | 11.29                                 | 0.66               | 25.62                                     | 44.1 wt %                                                     | Yes                        |
| Ex 5   | 1.2% UCARE™ JR 400            | 54.5                                   | 10.59                      | 11.25                        | 51.5 wt %                                    | 51.5 wt %                     | 13.30           | 7.16                                  | 1.35               | 17.75                                     | 40.3 wt %                                                     | Yes                        |
| Ex 6   | 0.4% UCARE™ JR 400            | 54.5                                   | 0.87                       | 2.10                         | 70.7 wt %                                    | 70.7 wt %                     | 1.58            | 0.93                                  | 0.70               | 1.8                                       | 51.7 wt %                                                     | Yes                        |
| Ex 7   | 0.4% UCARE™ JR 400            | 54.5                                   | 0.82                       | 1.58                         | 65.8 wt %                                    | 65.8 wt %                     | 1.57            | 0.83                                  | 0.53               | 1.65                                      | 50.3 wt %                                                     | Yes                        |
| Ex 8   | 0.4% UCARE™ JR 400            | 54.5                                   | 0.89                       | 2.22                         | 71.4 wt %                                    | 71.4 wt %                     | 1.51            | 0.49                                  | 0.78               | 1.38                                      | 35.5 wt %                                                     | Yes                        |
| Ex 9   | 2.0% UCARE™ JR 125            | 21.0                                   | 11.14                      | 13.55                        | 54.9 wt %                                    | 54.9 wt %                     | 26.21           | 5.83                                  | 1.38               | 16.97                                     | 34.4 wt %                                                     | Yes                        |

<sup>1</sup>UCARE Solution percentage is the wt % of the hydroxyethylcellulose polymer with a quaternary ammonium cation group, based on the total weight of the aqueous solution.

<sup>2</sup>The PUD Solids Content is the solids content of the PUD, based on the total weight of the PUD.

<sup>3</sup>The Modified Textile Component wt % Aqueous Solution is the wt % of aqueous solution present in the modified textile component before drying, based on the total weight of the modified textile component.

<sup>4</sup>The Polyurethane Pick-Up is the amount in grams (g) of polyurethane present in the synthetic leather after drying.

<sup>5</sup>The Synthetic Leather Polyurethane wt % After Drying is the wt % of polyurethane that is present in the synthetic leather after drying, based on the total weight of the synthetic leather. NM = not measured

Comparative Sample 1 and Comparative Sample 2, each of which are prepared without contacting a textile with an aqueous solution containing a cationic hydroxyethylcellulose polymer to form a modified textile component, contain no pores in the polyurethane matrix. Consequently, Comparative Sample 1 and Comparative Sample 2 are not suitable for synthetic leather applications.

Examples 3-9, which are prepared by first contacting a textile with an aqueous solution comprising a cationic hydroxyethylcellulose polymer to form a modified textile component; then, impregnating the modified textile component with a PUD externally stabilized with an anionic surfactant; precipitating the polyurethane in the modified textile component; and forming a synthetic leather, advantageously exhibit good coagulation (as evidenced by the formation of pores in the polyurethane matrix). Further, the polyurethane matrix of Examples 3-9 each exhibits a uniform distribution of pores throughout the polyurethane

We claim:

1. A process comprising:
  - first, contacting a textile with an aqueous solution consisting of (i) a cationic hydroxyethylcellulose polymer, (ii) water, and (iii) optionally silicone oil to form a modified textile component;
  - subsequently, impregnating the modified textile component with an aqueous polyurethane dispersion externally stabilized with an anionic surfactant; and
  - precipitating, in the absence of a free inorganic salt, the polyurethane in the modified textile component.
2. The process of claim 1 comprising (iv) forming a synthetic leather.
3. The process of claim 1 comprising selecting a cationic hydroxyethylcellulose polymer that is a hydroxyethylcellulose polymer with a quaternary ammonium cation group.
4. The process of claim 3 comprising selecting a cationic hydroxyethylcellulose polymer having a weight average molecular weight (Mw) from 100,000 Dalton to 3,000,000 Dalton.

## 25

5. The process of claim 4 wherein cationic hydroxyethylcellulose polymer has a Structure (A)



wherein

n is an integer from 200 to 10,000,

x is an integer from 0 to 30, and

y is an integer from 1 to 10.

## 26

6. The process of claim 5 comprising

(i) first, contacting the textile with an aqueous solution consisting of (i) the cationic hydroxyethylcellulose polymer, (ii) water, and (iii) silicone oil to form a modified textile component.

7. The process of claim 5 comprising

(i) first, contacting the textile with an aqueous solution consisting of (i) the cationic hydroxyethylcellulose polymer, and (ii) water to form a modified textile component.

10 8. The process of claim 1 comprising selecting an anionic surfactant that is a sulfonate surfactant.

9. The process of claim 1 comprising maintaining, during the impregnating, a Cation:Anion Ratio from 0.1 to 10.

15 10. The process of claim 1 comprising drying the modified textile component before impregnating the modified textile component with the aqueous polyurethane dispersion.

11. The process of claim 1 comprising forming a synthetic leather comprising from 20 wt % to 70 wt % polyurethane.

12. The process of claim 1 wherein the aqueous solution comprising a cationic hydroxyethylcellulose polymer is void of organic solvent.

20 13. The process of claim 12 wherein the aqueous polyurethane dispersion is void of organic solvent.

\* \* \* \* \*